

1

3,206,403

MINERAL OIL CONCENTRATES CONTAINING  
NON-ASH-FORMING OIL ADDITIVES  
Bobby W. Malone, East Norwalk, Conn., and Julian G.  
Ryan, Wood River, Ill., assignors to Shell Oil Company,  
New York, N.Y., a corporation of Delaware  
No Drawing. Filed July 22, 1964, Ser. No. 384,534  
7 Claims. (Cl. 252—49.9)

This application is a continuation-in-part of our co-pending applications Serial No. 112,752, filed May 26, 1961, Serial No. 863,098, filed December 31, 1959, and Serial No. 776,419, filed November 26, 1958, all of which are now abandoned.

The present invention relates to mineral oil concentrates of certain non-ash-forming additive mixtures, which concentrates are compatible with and stably dispersible in any liquid mineral lubricating oil which may be neat or compounded.

It is known that certain oil-soluble non-ash-forming nitrogen-containing polymeric detergents in which the nitrogen-containing groups may be amido groups such as vinyl pyrrolidones, in conjunction with a p,p'-methylene bisphenol



where the R's are alkyl groups, preferably tertiary alkyl groups, when added in small amounts to lubricating oils impart to the oil a high degree of stability and excellent detergency. However, it has been observed that the type of oil to which these additives are added is critical if separation of the additives from the oil is to be prevented particularly when oils containing the additive mixture are stored in concentrated form and later blended with conventional lubricating stocks such as commercial mineral lubricating oils, which are neat or compounded with conventional oil additives such as sulfonates, organic phosphites, phosphates, phosphonates or their thio-derivatives, phenates, thiocarbamates, aromatic or aliphatic amines, etc., to give a finished lubricant.

A principal object of the invention is to provide a mineral oil concentrate containing certain polymeric nitrogen-containing detergents and p,p'-methylene bisphenols which are stably dispersible in any lubricating oil. Another object of the invention is to provide a mineral oil concentrate containing said two additives which concentrate is dispersible in conventional mineral lubricating oils and are stably suspended or dispersed therein both during storage and use. Still another object of the invention is to provide a mineral oil concentrate containing said two additives which when added to conventional mineral lubricating oil would meet and pass revised MIL-L-6082B and MIL-L-22851 specifications. Another object of the present invention is to provide a mineral oil concentrate containing substantial amounts of each of said two additives which when added to lubricating oils would result in excellent aircraft and automotive lubricants. Other objects will be apparent from the following description.

It has now been discovered that the additive combination of an oil-soluble polymeric detergent of a copolymer of a vinyl pyrrolidone and an acrylate ester and p,p'-methylene bisphenols as represented by Formula A can be stably suspended or dispersed in amounts of from about

2

15%, preferably 20% to about 60% or higher preferably 40% of the polymeric detergent and from about 3%, preferably 5% to about 20% or higher, preferably about 15% by weight of the p,p'-methylene bisphenol, in a highly refined East Texas raffinate mineral oil fraction containing from 20 to 30 carbon atoms, essentially free of sulfur compounds and tri-, tetra-, penta-, hexaaromatics but a substantial portion of which, namely 10% to 30% are mono- and diaromatics and the balance being saturates which includes alkanes, condensed and non-condensed cycloalkanes, said oil having a molecular weight range of from 280 to 500 and a VI of from 75 to 100. It is preferred that the weight ratio of the polymer to the bisphenol in the concentrate be from 15:1 to about 5:1, preferably from about 10:1 to about 8:1, respectively. East Texas base mineral oil concentrates of this type can be added to any type of mineral oil in any desired concentration without worry of separation, compatibility, interaction or other undesirable side effects both during storage or use.

The detergent copolymers useful in forming concentrates of the present invention include copolymers of vinyl pyrrolidone and polymerizable acrylates and methylacrylates such as N-vinyl pyrrolidone and C<sub>6</sub>—C<sub>20</sub> alkyl acrylate e.g. lauryl methylacrylate or similar copolymers as described in Belgian Patent 550,422 and British Patent 808,664, and mixtures thereof. Acrylate-vinyl pyrrolidone copolymers are sold by Rohm and Haas under the designations Acryloid 315X or 917 or 966 and are copolymers of N-vinyl pyrrolidone and lauryl methacrylate of varying molecular weight of from about 100,000 to about 650,000.

The long chain acrylate esters used in the preparation of the copolymers include the esters of acrylic acids and long chain aliphatic alcohols. Examples of the acrylic acids include acrylic acid and the alpha-substituted acrylic acids such as methacrylic acid, ethacrylic acid, alpha-phenyl acrylic acid, alpha-cyclohexyl acrylic acid and chloroacrylic acid. The long-chain aliphatic alcohols used in the esterification of these acids may be exemplified by decyl, lauryl, cetyl, stearyl, eicosanyl, nonadecanyl alcohols and the like and mixtures thereof. Particularly preferred esters to be used are the acrylic acid and methacrylic acid esters of aliphatic monohydric alcohols, and especially alkyl alcohols, containing from 14 to 20 carbon atoms.

Specific examples of these long chain acrylic acid esters include, among others, decyl acrylate, lauryl acrylate, stearyl acrylate, decyl methacrylate, lauryl methacrylate, cetyl methacrylate, stearyl methacrylate, eicosanyl acrylate, docosanyl acrylate, and the like, and mixtures thereof.

As noted, a mixture of one and preferably two or more of these long chain acrylate esters can be used in making the copolymers. Illustrative examples of these ester mixtures include, among others, dodecyl methacrylate/tetradecyl methacrylate, tetradecyl acrylate/octadecyl methacrylate, decyl methacrylate/octadecyl methacrylate; tetradecyl methacrylate/hexadecyl methacrylate; tetradecyl methacrylate/octadecyl methacrylate; dodecyl methacrylate/eicosanyl acrylate, and the like.

In the mixtures, it is highly desirable to have a substantial difference in the number of carbon atoms of the alcohol portion. Particularly superior results are obtained when one of the acrylate esters is a C<sub>10</sub> to C<sub>14</sub> acrylate ester and the other is a C<sub>16</sub> to C<sub>20</sub> acrylate ester.

In the mixtures, the different long chain acrylate esters are employed in mol ratios from 1:4 to 4:1. The su-

terior copolymers are obtained when the higher ester, e.g., those having from 10 to 20 carbon atoms in the alcohol portion, and the lower esters, e.g., those having from 10 to 14 carbon atoms in the alcohol portion are combined in a mol ratio varying from 1:1 to 1:3.

Copolymers of the present invention which have the superior properties above are those having molecular weights between 50,000 and 2,500,000 as determined by the light scattering technique described in Chem. Rev., vol. 40, page 319 (1948). Preferably, the molecular weights range from about 75,000 to 1,000,000 and more preferably from 100,000 to 650,000.

The following examples illustrate the preparation of suitable polymers for use in compositions in accordance with the invention. Unless otherwise specified, parts disclosed in the examples are parts by weight.

In the examples, the molecular weights were determined by light scattering method and the ratio of vinyl pyrrolidones to alkyl ester was determined by analysis for nitrogen.

#### EXAMPLE I

A mixture of about 2 mols of lauryl methacrylate, 1 mol of N-vinyl pyrrolidone and 0.5% by weight of benzoyl peroxide was reacted in a suitable reaction vessel for a period of about 10 hours at about 65° C. The polymer was then dispersed in benzene and thereafter precipitated with a mixture of acetone and methanol. A copolymer of lauryl methacrylate/N-vinyl pyrrolidone having a nitrogen content of 2.20% by weight and a molecular weight in excess of 250,000 was recovered. The polymer contained the monomer units essentially in the ratio as provided in the mixture; it had an alkane chain of about 2400 carbon atoms carrying about 800 lauryloxyformyl groups and about 400 butyrolactam groups.

#### EXAMPLE II

A copolymer of lauryl methacrylate and N-vinyl pyrrolidone was prepared by the method of Example I with the same monomer ratio but in which 0.75% by weight of alpha,alpha-azodiisobutyronitrile was used as the catalyst. The molecular weight of the polymer was around 225,000.

#### EXAMPLE III

A terpolymer of stearyl methacrylate/lauryl methacrylate/N-vinyl pyrrolidone in the mol ratio of 2.8/5.6/1, respectively, was prepared essentially by the method of Example I using 0.2% alpha,alpha-azodiisobutyronitrile as catalyst and the reaction time was 48 hours. The polymeric product was oil-soluble and had an average molecular weight over  $1 \times 10^6$  as determined by the light scattering technique.

Other representative copolymers useful in compositions of this invention include those identified below in which the monomeric units are present in the mol ratios of 1:1, 1:2, 1:4, 1:6, of the monomer, one to the other, and preferably of N-vinyl pyrrolidone to ester, respectively, said copolymers having a molecular weight in excess of 50,000: N-vinyl pyrrolidone/octyl methacrylate, N-vinyl-3-methyl pyrrolidone/cetyl methacrylate, N-vinyl pyrrolidone/stearyl methacrylate, N-vinyl pyrrolidone/stearyl acrylate, N-vinyl-3,3-dimethyl pyrrolidone/lauryl methacrylate, N-vinyl pyrrolidone/stearyl methacrylate/cetyl methacrylate, N-vinyl-3-methyl pyrrolidone-stearyl methacrylate/lauryl methacrylate, and mixtures thereof.

The methylene bisphenol represented by the above structural Formula A can be prepared by any suitable means such as by reacting a di-tertiary alkyl phenol with formaldehyde in the presence of an organic solvent such as heptane and an acidic catalyst such as sulfuric acid. Another method is to react the di-tertiary alkyl phenol with formaldehyde in the presence of an acid catalyst in an aqueous medium. The general method of preparing

these compounds is well known in the art and does not form a part of the present invention. Compounds of this type include 4,4'-methylene bis(2,6-di-tertiarybutyl phenol), 4,4'-methylene bis(2,3-di-tertiarybutyl phenol), 4,4'-methylene bis(2,5-di-tertiarybutyl phenol), 4,4'-methylene bis(3,5-di-tertiarybutyl phenol), 4,4'-methylene bis(2,6-di-tertiaryoctyl phenol), 4,4'-methylene bis(2-tertiarybutyl, 6-tertiaryoctyl phenol), and mixtures thereof.

10 The East Texas raffinate mineral oil base used to form the concentrate containing the two essential additives described above not only function as a carrier for the additives when from about 10% to about 80% of the concentrate is added to any mineral lubricating oil to form stable finished lubricating oil compositions. The East Texas raffinate fraction used in forming the concentrate is a highly refined East Texas raffinate fraction containing from about 20 to about 30 carbon atoms and is essentially 15 free of sulfur, nitrogen and oxygen constituents as well as higher polyaromatics such as the tri-, tetra-, penta-aromatics, e.g., the phenanthrenes, anthracenes, dibenzothiophenes, chrysenes, pyrenes, etc., and resins, but which is rich in mono- and diaromatics (10-30%) and saturates 20 which include alkanes, non-condensed and condensed cycloalkanes totaling 70-90% of the hydrocarbon mixture. The VI of such raffinate fractions ranges from 75 to 100 and the molecular weight varies from about 280 to about 500. East Texas raffinate fractions used in forming the concentrate of the present invention may be obtained by solvent (phenol or furfural) extraction of suitable East Texas distillates having a viscosity range of 150 to 400 SUS at 100° F. A typical East Texas distillate (250 SUS 100° F.) from which, by phenol extraction, 25 suitable raffinate fractions can be obtained ranging in VI from 75 to 93 on analysis contained the following hydrocarbon types.

Table I

#### COMPONENTS OF 250 EAST TEXAS (ET) DISTILLATE

| Components, percent wt.:        | Distillate |
|---------------------------------|------------|
| n-Alkanes -----                 | 13.1       |
| Isoalkanes -----                | 10.8       |
| Noncondensed cycloalkanes ----- | 26.7       |
| Condensed cycloalkanes -----    | 16.9       |
| Total saturates -----           | 67.5       |
| Monoaromatics -----             | 13.7       |
| Di aromatics -----              | 5.8        |
| Tri aromatics -----             | 4.2        |
| Tetra aromatics -----           | 2.1        |
| Penta aromatics -----           | 1.5        |
| Hexa aromatics -----            | 0.5        |
| Total sulfur compounds -----    | 4.7        |
| Total -----                     | 100.0      |
| Sulfur analysis, percent wt.:   |            |
| Thiophenes-----                 |            |
| Benzene-----                    | 1.6        |
| Tri aromatics-----              | 0.6        |
| Tetra aromatics-----            | 0.3        |
| Penta aromatics-----            |            |
| Other sulfur compounds-----     | 2.2        |
| Total -----                     | 4.7        |

70 The raffinate fraction obtained from the above distillate by phenol extraction followed by methyl ethyl ketone-toluene treatment contains the following components and this East Texas (ET) is an excellent carrier for the additives of the present invention whereas raffinates obtained from other sources, e.g., West Texas-Ellenberger (WTE) or Oklahoma fraction (OC) are unsuited and their compounds are shown in Tables III and IV.

Table II

## COMPONENTS OF ET 250 RAFFINATE

| Components, percent wt.:      | Raffinate |
|-------------------------------|-----------|
| n-Alkanes                     | 17.3      |
| Isoalkanes                    | 15.8      |
| Noncondensed cycloalkanes     | 34.0      |
| Condensed cycloalkanes        | 18.4      |
| Total saturates               | 85.5      |
| Monoaromatics                 | 10.4      |
| Diaramatics                   | 2.7       |
| Triaromatics                  | 0.8       |
| Tetraaromatics                | 0.2       |
| Pentaaromatics                | —         |
| Hexaaromatics                 | —         |
| Total sulfur compounds        | 0.4       |
| Total                         | 100.0     |
| Sulfur analysis, percent wt.: |           |
| Thiophenes—                   |           |
| Benz—                         | 0.2       |
| Triaromatics                  | 0.1       |
| Tetraaromatics                | 0.1       |
| Pentaaromatics                | —         |
| Other sulfur compounds        | —         |
| Total                         | 0.4       |

Table III

## COMPONENTS OF WEST TEXAS-ELLENBERGER (WTE) 250 DISTILLATE AND RAFFINATE

|                               | Distillate | Raffinate |
|-------------------------------|------------|-----------|
| Components, Percent wt.:      |            |           |
| n-Alkanes                     | 8.0        | 13.5      |
| Isoalkanes                    | 37.6       | 37.8      |
| Noncondensed Cycloalkanes     | 15.8       | 19.0      |
| Condensed Cycloalkanes        |            |           |
| Total Saturates               | 61.4       | 70.3      |
| Monaaromatics                 | 18.2       | 19.0      |
| Diaramatics                   | 6.7        | 5.5       |
| Triaromatics                  | 4.3        | 2.4       |
| Tetraaromatics                | 2.6        | 0.9       |
| Pentaaromatics                | 2.0        | 0.4       |
| Hexaaromatics                 | 0.2        | —         |
| Total Sulfur Compounds        | 4.6        | 1.5       |
| Total                         | 100.0      | 100.0     |
| Sulfur Analysis, Percent wt.: |            |           |
| Thiophenes—                   |            |           |
| Benz—                         | 1.5        | 0.7       |
| Triaromatics                  | 0.7        | 0.3       |
| Tetraaromatics                | 0.2        | 0.1       |
| Pentaaromatics                | 0.1        | —         |
| Other Sulfur Compounds        | 2.1        | 0.4       |
| Total                         | 4.6        | 1.5       |

Table IV

## COMPONENTS OF OKLAHOMA (OC) 250 DISTILLATE AND RAFFINATE

|                               | Distillate | Raffinate |
|-------------------------------|------------|-----------|
| Components, Percent wt.:      |            |           |
| n-Alkanes                     | 15.1       | 18.2      |
| Isoalkanes                    | 32.6       | 39.6      |
| Noncondensed Cycloalkanes     | 17.6       | 20.4      |
| Condensed Cycloalkanes        |            |           |
| Total Saturates               | 65.3       | 78.2      |
| Monaaromatics                 | 15.9       | 14.0      |
| Diaramatics                   | 6.1        | 3.9       |
| Triaromatics                  | 4.3        | 1.8       |
| Tetraaromatics                | 1.5        | 0.6       |
| Pentaaromatics                | 1.2        | 0.1       |
| Hexaaromatics                 | 0.4        | —         |
| Total Sulfur Compounds        | 5.3        | 1.4       |
| Total                         | 100.0      | 100.0     |
| Sulfur Analysis, Percent wt.: |            |           |
| Thiophenes—                   |            |           |
| Benz—                         | 0.4        | 0.3       |
| Triaromatics                  | 0.3        | 0.2       |
| Tetraaromatics                | 1.0        | 0.4       |
| Pentaaromatics                | 1.4        | 0.3       |
| Other Sulfur Compounds        | 2.2        | 0.2       |
| Total                         | 5.3        | 1.4       |

The East Texas raffinate (Table II) shown above is excellent for forming the concentrate of the present invention. However, oil fractions in the same viscosity range as the East Texas raffinate such as obtained from West Texas-Ellenberger (WTE) or Poso Coalinga or Oklahoma crudes shown in Tables IV and V are unsuited for forming the concentrates of the present invention since such concentrates when blended with conventional lubricating oils such as SAE 5W to 90 mineral lubricating oils or aviation oils of the so-called 1100 or 1065 grade aircraft oils or the 80 or 100 viscosity grade aviation oils present a compatibility problem particularly when such oils contain conventional antioxidants, e.g., alkyl phenols, aromatic amines, or metallic detergents, e.g., oil-soluble metal sulfonates, phenates, wear inhibitors, e.g., metal organic phosphates, thiocarbamates, etc.

A preferred embodiment of the present invention is to blend 10-20% of concentrate with an East Texas lubricating oil in the viscosity range (SAE 5W-90) so as to form the final or finished lubricant and if desired add to the concentrate or the finished product a small amount (0.01-3%, preferably 0.1-1%) of a partial or full ester of an organic phosphorus compound. Phosphorus compounds of this type include alkyl, cycloalkyl, alkaryl, aralkyl, and aryl phosphites, phosphates, phosphonates, and their thio-derivatives, such as  $C_{8-18}$  alkyl phosphites, e.g., di- and tributyl, octyl, lauryl, stearyl, cyclohexyl, benzyl, cresyl, phenyl phosphites or phosphates, as well as their thio-derivatives;  $P_2S_5$ -terpene reaction product,  $P_2S_5$ -pine oil reaction product; dibutyl methane-phosphonate, dibutyl trichloromethane phosphonate, dibutyl monochloromethane phosphonate, dibutyl chlorobenzene phosphonate, and the like. The esters of pentavalent phosphorus acids such as diphenyl, di-cresyl, triphenyl, tricresyl, trilauryl and tristearyl ortho phosphates,  $P_2S_5$ -terpene reaction products and mixtures thereof are preferred.

Concentrates illustrating the present invention are shown below.

Table V

| Concentrate, percent wt.:                                 | A  |
|-----------------------------------------------------------|----|
| Percent East Texas 250/100° F. SUS raffinate <sup>1</sup> | 10 |
| Percent Example I copolymer                               | 67 |
| Percent 4,4'-methylene bis(2,6-di-tertbutylphenol)        | 30 |

| PROPERTIES              |      |
|-------------------------|------|
| Vis. SSU at:            |      |
| 100° F                  | 2700 |
| 210° F                  | 346  |
| Pour point, °F          | -20  |
| Gravity, °API           | 28.2 |
| Storage Stability, Days | >50  |

## PROPERTIES OF CONCENTRATES IN AIRCRAFT OIL 1100

|                             | MIL Spec 6082B |
|-----------------------------|----------------|
| 55 Vis. SSU at:             |                |
| 100° F                      | 1298           |
| 210° F                      | 115            |
| Viscosity index             | 111            |
| Ash, percent wt.            | 0.0025 max.    |
| Neutralization No.          | 0.10 max.      |
| Neutral                     | Neutral        |
| Precipitation No.           | 0              |
| Copper corrosion            | 1A             |
| Sulfur, percent wt.         | 0.5 max.       |
| Saponification No.          | 0.5 max.       |
| Flash, COC, °F              | 495            |
| Fire, COC, °F               | 560            |
| Cloud point, °F             | 40             |
| Pour point, °F              | -10            |
| Diluted pour point, °F      | B-65           |
| Carbon residue, percent wt. | 1.2 max.       |
| Gravity, °API               | 27.8           |
| Storage stability, days     | >50            |

<sup>1</sup> Note Table II.

<sup>2</sup> Viscosity specification set by Navy for 1100-grade aircraft oils containing mineral oil concentrate.

The above concentrate A made with different stocks such as Oklahoma or West Texas in the same viscosity range or blended with a 1100 aircraft oil would on storage separate in 10-15 days.

Examples of other concentrates of the present invention are shown in Table VI:

Table VI

| Concentrate, percent wt.                          | B<br>10 | C<br>10   | D<br>10   | E<br>20   | F<br>20   | G<br>40                                      |
|---------------------------------------------------|---------|-----------|-----------|-----------|-----------|----------------------------------------------|
| Example I, percent                                | 60      |           |           |           |           | 30.                                          |
| Example II, percent                               | 30      |           |           | 40        |           |                                              |
| Example III, percent                              |         | 30        |           |           | 50        |                                              |
| 4,4'-methylene bis(2,6-ditertbutylphenol) percent | 6       | 3         | 3         |           | 5         | 3.                                           |
| 4,4'-methylene bis(2,6-octylphenol) percent       |         |           |           | 5         |           |                                              |
| Tricresyl phosphate                               |         |           |           |           | 1.5       |                                              |
| Dicresyl phosphate                                |         |           |           |           | 1         |                                              |
| Dimethyl silicone                                 | Balc    | 50 p.p.m. | 50 p.p.m. | 25 p.p.m. | 25 p.p.m. | 50 p.p.m.                                    |
| ET 250/100, percent                               | Balc    | Balc      | Balc      | Balc      | Balc      | Balc                                         |
| ET 350/100, percent                               |         |           |           |           |           | (50/50 mixture of ET250 and ET350 at 100°F). |

Concentrates B, C and D diluted with 90% of 1100 aircraft oil were storage stable for over 50 days; Concentrates E and F diluted with 80% West Texas-Ellenberger oil (250/100° F.) were stable for over 50 days and Concentrate G diluted with 60% Oklahoma 250/100° F. mineral lubricating oil was stable for over 50 days and these compositions passed all requirements of MIL-L-6085B and MIL-L-22851 specification. On the other hand, when in these concentrates the East Texas raffinate was substituted with different base stocks such as a Poso-Coalinga or WTE lube oil stock and these concentrates were diluted with 1100 aircraft oil, or WTE, or Oklahoma lube oil stocks, as indicated in Table VI, the storage stability was reduced 50 to 75%, and these compositions failed to pass the above specification requirements.

Concentrates of the present invention may be used as lubricants per se. When diluted with suitable mineral oils as described, the finished products possess improved storage, detergency and oxidation stability.

We claim as our invention:

1. A mineral oil additive concentrate consisting essentially of a mixture of from about 15% to about 60% by weight of a copolymer of vinyl pyrrolidone and a  $C_{12-18}$  alkyl methacrylate and from 3% to 20% by weight of 4,4'-methylene bis(2,6-dialkylphenol) and the balance being an East Texas mineral lubricating oil raffinate fraction consisting essentially of from 10% to 30% by weight of mono- and diaromatics and 90-70% by weight of saturates.

2. A mineral oil additive concentrate consisting essentially of a mixture of from about 15% to about 60% by weight of a copolymer of vinyl pyrrolidone and lauryl methacrylate and from about 3% to about 20% by weight of 4,4'-methylene bis(2,6-ditertbutyl phenol) and the balance being an East Texas mineral lubricating oil raffinate fraction consisting essentially of from 10% to 30% by weight of mono- and diaromatics and 90-70% by weight of saturates.

3. A mineral oil additive concentrate consisting essentially of a mixture of from 20 to 40% by weight of a copolymer of vinyl pyrrolidone and a  $C_{12-18}$  alkyl meth-

acrylate and from 5 to 15% by weight of 4,4'-methylene bis(2,6-dialkylphenol) and the balance being an East

Texas mineral lubricating oil raffinate fraction consisting essentially of 10 to 30% by weight of mono- and diaromatics and 90-70% by weight of saturates.

25 4. A mineral oil additive concentrate consisting essentially of a mixture of from 20 to 40% by weight of a copolymer of vinyl pyrrolidone and lauryl methacrylate and from 5 to 15% by weight of 4,4'-methylene bis(2,6-ditertbutyl phenol) and the balance being an East Texas mineral lubricating oil raffinate fraction consisting essentially of 10 to 30% by weight of mono- and diaromatics and 90-70% by weight of saturates.

30 5. A mineral oil additive concentrate consisting essentially of a mixture of about 30% by weight of a copolymer of vinyl pyrrolidone and lauryl methacrylate and about 3% by weight of 4,4'-methylene bis(2,6-ditertbutyl phenol) and the balance being an East Texas mineral lubricating oil raffinate fraction consisting essentially of 10 to 30% by weight of mono- and diaromatics and 90-70% by weight of saturates.

35 6. A mineral oil additive concentrate consisting essentially of a mixture of about 60% by weight of a copolymer of vinyl pyrrolidone and lauryl methacrylate and about 6% by weight of 4,4'-methylene bis(2,6-ditertbutyl phenol) and the balance being an East Texas mineral lubricating oil raffinate fraction consisting essentially of 10 to 30% by weight of mono- and diaromatics and 90-70% by weight of saturates.

40 7. The concentrate of claim 4 containing from 1 to 50 5% by weight of tricresyl phosphate.

#### References Cited by the Examiner

##### UNITED STATES PATENTS

|              |      |                       |            |
|--------------|------|-----------------------|------------|
| 55 2,498,628 | 2/50 | Cyphers et al. -----  | 252—49.8 X |
| 2,807,653    | 9/57 | Filbey et al.         |            |
| 2,886,523    | 5/59 | Claridge et al. ----- | 208—18 X   |
| 3,030,303    | 4/62 | Ryan -----            | 252—51.5 X |

##### FOREIGN PATENTS

|            |       |                |
|------------|-------|----------------|
| 60 808,665 | 2/59  | Great Britain. |
| 851,588    | 10/60 | Great Britain. |

DANIEL E. WYMAN, Primary Examiner.